

## UNITED STATES PATENT OFFICE

HUGH S. COOPER, OF CLEVELAND, OHIO, ASSIGNOR TO KEMET LABORATORIES COMPANY, INC., A CORPORATION OF NEW YORK

## PRODUCING VACUUMS

No Drawing.

Application filed December 31, 1929. Serial No. 417,825.

The invention relates to the production of high vacuums for any purpose, but particularly in hot cathode devices such as the tubes or valves used in radio communication.

5 In the prevailing practice, electron tubes are evacuated by pumping to a convenient degree of exhaustion, and then subjecting the residual gases to the action of a clean-up agent, which, it is believed, fixes the residual 10 gases by both chemical and physical action. Magnesium is the usual clean-up agent, but other substances, for example the metals barium and strontium, give higher vacuums under certain conditions. In attempting to 15 substitute these latter metals for magnesium, difficulties are encountered because the metals require higher temperatures than magnesium to cause them to "flash", that is to begin to react rapidly with the gases present.

20 The usual method of flashing the clean-up agent is to introduce it in solid form into the envelope, then seal the envelope either temporarily or permanently, and then bring the envelope into the field of a coil in which high- 25 frequency alternating current flows; and it is found that the equipment available, designed for flashing magnesium, may not have enough power to flash barium and other very active agents within the time allotted to this 30 operation in the semi-automatic machines used in making thermionic tubes. In the present large-scale manufacture of tubes, it is of course desirable to carry out each operation as rapidly as possible.

35 An object of the invention is to facilitate the flashing of such agents as barium and strontium, and to adapt them to the equipment and schedules now employed with magnesium. This is accomplished by alloying the 40 barium or strontium with magnesium in such proportions as to produce stable alloys containing effective quantities of the former metals, powdering the resulting brittle alloys and compressing the powders which are self- 45 bonding, into pellets of the desired size.

The invention will be described more particularly hereinafter by reference to alloys of barium with magnesium.

50 Magnesium and barium alloy in all proportions, and certain of the alloys have been

found to be relatively stable in the air. It will be recognized that it is impossible to differentiate sharply between compositions which are stable in air and those which are not, especially since the action of the air 55 varies with its humidity, but it may be stated that stability falls off with increasing barium content, and that alloys containing up to about 30% of barium are fairly stable in air. Alloys which are unstable in air are also use- 60 ful, but they must be protected from pro- longed exposure to air. As little as 10% of magnesium alloyed with barium will sub- stantially lower the energy requirements for 65 flashing the getter, while as little as 5% of barium increases the thoroughness of the clean-up. The alloys of barium and mag- nesium which are most suitable for my pur- 70 pose have little ductility as a rule and cannot be readily drawn into wire or other attenu- ated forms. Some of the alloys are quite brittle. This property does not constitute 75 a serious objection as I have found that the powdered alloys have self bonding proper- ties and can be readily agglomerated, as by pressing into pellets. Appropriate binders may be used if desired.

The pellets of the powdered alloy as stated are stable in air and readily may be handled without objectionable contamination by va- 80 porizable impurities.

Barium-magnesium alloys can be easily prepared by fusing the ingredients in an inert atmosphere, such as argon or helium, in a suitable vessel, for example a crucible of 85 commercially carbon-free iron. For pure barium I may substitute any barium alloy which is free from substances detrimental to a gas clean-up agent. Similarly, strontium 90 alloys can be substituted for pure strontium.

I claim:

1. The method of cleaning up gases which comprises introducing into an envelope a pellet of powdered alloy consisting essen- 95 tially of magnesium and an alkaline earth metal, the latter constituting from about 5% to about 30% of the alloy, mechanically evacuating the envelope, and flashing the alloy.

2. The method of cleaning up gases which 100

comprises introducing into an envelope a pellet of powdered alloy consisting essentially of magnesium and barium, the latter constituting from about 5% to about 30% of the alloy, mechanically evacuating the envelope, and flashing the alloy.

3. As a clean-up agent, a pellet of a powdered alloy of magnesium and from about 5% to about 30% of an alkaline earth metal.

10 4. As a clean-up agent, a pellet of a powdered alloy of magnesium and from about 5% to about 30% of barium.

In testimony whereof, I affix my signature.  
HUGH S. COOPER.

15

20

25

30

35

40

45

50

55

60

65